

# UNITED STATES PATENT OFFICE.

CHARLES ALFRED CARLES DE CAUDEMBERG, OF NICE-GARE, FRANCE.

## PAVING COMPOSITION AND PROCESS OF MAKING THE SAME.

1,395,396.

Specification of Letters Patent.

Patented Nov. 1, 1921.

No Drawing.

Application filed January 15, 1921. Serial No. 437,587.

To all whom it may concern:

Be it known that I, CHARLES ALFRED CARLES DE CAUDEMBERG, a citizen of France, residing at Nice-Gare, in the Province of 5 Alpes-Maritimes, Republic of France, have invented a new and useful Paving Composition and Process of Making the Same, of which the following is a specification.

This invention relates to a paving 10 pound and process of making the same. It has for its object the improvement of processes of preparing combinations of all kinds of bituminous substances with rubber, the bitumens being in the form of asphalt, asphaltic rock, residues of the distillation of 15 oils of naphtha and petroleum, etc.

It is well known to those skilled in the art, that rubber dissolved in gasoline can be combined with bitumen, impregnating 20 the pulverized calcareous grains of the asphalt (asphaltic rock) to form a sticky mass which permits the agglomeration of the asphalt by simple compression.

The above process, which practically consists of diffusing through a mass of powdered asphalt, a solution of rubber in gasoline or like solvent and effecting the compression before the solvent evaporates, presents many defects. The solvent not only 25 does not dissolve more than a small proportion of rubber, but certain elements of the gum remain insoluble and form a large deposit. Besides, the special qualities of the rubber, especially its glutinous quality, are 30 visibly altered and this alteration becomes more marked with time. Again, the dissolving action of the solvent on the bitumen is very slow, and this action (indispensable for the combination) is further retarded 35 because of the gum content of the solution. Finally, the boiling point of this solvent, and its volatilization is all the more rapid, since it is promoted by mixing it with the powder, which enlarges the evaporating surface. 40

The result is that the quantity of rubber that can be incorporated in the asphalt, under these conditions, is strictly limited. It cannot exceed 30 or 40 grams per 50 kilograms of powder, and even then its combination with the bitumen is incomplete.

Although with this weak proportion the compression can be effected and the cohesion of certain kinds of asphalt powders can be insured, (which powders on account of their binding nature and a special addition of bitumen are particularly adapted to the process,) a number of other powders do not lend themselves to this method, either because they have too great content of bitumen or 55 because the character of the bitumen or that of the calcareous grains impregnated by it offers more resistance to the action of the solvent. Consequently the combination does not take place to the degree necessary to insure the cohesion before the solvent evaporates. The same drawback occurs when the work takes place at a high temperature, which accelerates the volatilization. In 60 fact, the inherent advantages of the bitumen-rubber combination are very little developed, and have no appreciable effect. 65

The present invention permits the asphalt to be prepared for cold compression, under conditions insuring the entire incorporation 70 of rubber into bitumen to a much greater degree, the method being adapted to the composition of various kinds of asphalt and to changing temperatures. It also permits the use of the rubber-bitumen combination 75 in the preparation of all kinds of bitumens, residues and mixtures to be poured hot.

The result is a colloidal substance, indefinitely malleable and compressible, having powerful cohesive properties and offering a 80 fusion point much higher than bitumen. Thus there is made an industrial product entirely new, having the qualities of elasticity, impermeability and high resistance, entirely suited to cold compression and offering not only an important improvement 85 for current use in hot applications, but, in one form, permitting repaving of streets, etc., by a method different from those now employed. 90

The process of this invention consists in effecting the solutions by means of mixtures exercising a strong and rapid solvent action on both rubber and bitumen, offering a high boiling point and not injurious to the molecular constitution or the qualities of the dissolved elements. In certain proportions, 95 100

these mixtures become non-inflammable, an indispensable condition for hot preparations.

It has been found that such solvents can be obtained by adding to benzene or toluene, a tetrachlorethane in the proportion of 20% for cold preparations and 86% for hot ones, these proportions being capable of very slight variation.

10 The formulas of the solutions are:

|         |                    |           |
|---------|--------------------|-----------|
| A :—    | Tetrachlorethane   | 200 cc.   |
|         | Benzene or toluene | 800 cc.   |
|         | Rubber             | 25-50 gr. |
| 15 B :— | Tetrachlorethane   | 860 cc.   |
|         | Benzene or toluene | 140 cc.   |
|         | Rubber             | 50-75 gr. |

The solutions thus prepared are incorporated in the asphaltic and bituminous substances under various conditions, according to the method of application. The proportion of the quantities of rubber is in conformity with the composition of asphalt or mixtures employed, and with the various temperatures.

There are given below two practical examples of the process, one for the preparation and application of asphalt compressed cold, and the second for the preparation and 30 application of bitumens poured hot.

Example 1: Finely powdered asphalt is introduced into the barrel of a mixer. The apparatus being started the solution A is poured into the powder as the work of mixing progresses. The operation takes only a few minutes.

The quantity of solution to be mixed varies, according to its gum content, from 3 to 4 kilograms per 100 kilos of powder.

40 According to the special case, the quantity of rubber is regulated by employing solutions more or less strong, from 2.50% to 5%. Weak solutions are mixed very rapidly. To incorporate thick solutions, one 45 must effect the first impregnation with a light solution, which facilitates the absorption while softening the bitumen. Thus there can be used at first 500 to 1000 grams of a 2.50% solution and finally 2,000 grams 50 can be used with a 5% solution.

On leaving the mixer the material is spread out in a bed of uniform thickness on a concrete or cement foundation, already covered with light liquid cement. The material is compressed gradually but the use 55 of a roller for this purpose is not desirable because it displaces the material sidewise and interferes with its adherence to the cement.

60 For the manufacture of agglomerations of asphalt compressed by pressure, the preparation is the same as above. The pressure will be regulated to 300 kilos per square centimeter of surface.

65 Example 2: The preparation of bitumens

intended to be poured hot is effected by mixing with the solution B, the bitumen melted at a temperature slightly above its fusion point. The bitumen is introduced by pouring it in a fine stream, into the solution of cold rubber, the mass being constantly agitated.

The mixture thus obtained can be used in several ways:

First. To prepare asphalt poured in a 75 plastic state, the quantity of bitumen melted to be incorporated in the solution will be 5% of the quantity of asphalt to prepare, and the proportion of the solution B, 4 or 5 kilograms per 100 kilos of matter; the 80 proportion of rubber varying in respect to the fusion point desired, from 5% to 7.50%. The bitumen-rubber mixture having been brought to the temperature of 100-120 degrees, the plastic asphalt is introduced, 85 divided into successive portions, up to 150-180 degrees, to effect the cooking. During this operation proper provision can be made for collecting the vapors of the solvents to save them.

The product thus obtained can be adapted 90 to various applications. It can be added to sand or gravel. In this case, these substances are introduced, at the beginning of the cooking, in small quantities to prevent 95 cooling the mass. This preparation is advantageously utilized for all the purposes for which the ordinary mass can be used, as it has superior cohesion and resistance, and also greater elasticity. It can also be 100 used pure for certain kinds of work, which represents an entirely new application of poured asphalt, based on its high point of fusion, which insures stability at temperatures over 100 degrees, and does not involve 105 the use of hard substances, indispensable for the ordinary poured preparation.

In practice, the two processes can be combined by making a bed of the compound mixed with gravel and putting a layer of the 110 pure product thereon. The pure product is especially indicated for work that must be absolutely waterproof and yet must be elastic or yielding such as terraces, bridge heads, etc. The fused substance is simply poured 115 out on the surfaces to be covered and flattened by means of wooden planks or the like.

Second. Bitumen-rubber, prepared as described, can also be used for bituminous 120 concretes or asphalt-macadam. In this kind of roads, either the natural bitumens can be used, freed from all earthy matter, or the residues of the distillation of petroleum. Melted bitumen, mixed in the rubber solution in the proportion of 15-20 kilograms of solution per 100 of bitumen, is brought to the temperature of 150-180 degrees and poured directly, in the proportion of 10-12 kil. per square meter, on a rocky foundation 130

of 0.15-0.18 centimeters of thickness, previously placed on the earth and arranged evenly. The surface is covered with sand and a roller is passed over it.

5 The mixture of bitumen-rubber and pebbles may be made before it is applied. In certain instances, there is placed on this foundation a covering of the asphalt-plaster preparation, either pure or mingled with sand and fine gravel.

10 What is claimed is:—

1. A composition of matter for use as an industrial product, and resulting from the combination of bitumen with rubber, said rubber being contained in a solvent obtained by adding to benzene, tetrachlorethane in the proportion of about 20% for use when

cold and about 86% for use when hot, there being approximately 1-1.50 of rubber to 100 of bitumen.

20

2. A composition of matter for use as an industrial product, and resulting from the combination of bitumen with rubber in a proportion of approximately 1-1.50 of rubber to 100 of bitumen, said composition 25 having colloidal properties and a high point of fusion.

In testimony that I claim the foregoing as my own, I have hereto affixed my signature in the presence of two witnesses.

CHARLES ALFRED CARLES de CAUDEMBERG.

Witnesses:

DOUGLAS BOOTH,  
L. MOREAN.